

July 9, 1940.

L. V. FORMAN

2,207,218

PROCESS FOR REMOVAL OF DIRT FROM PULP

Filed Aug. 6, 1937

2 Sheets-Sheet 1



July 9, 1940.

L. V. FORMAN

2,207,218

PROCESS FOR REMOVAL OF DIRT FROM PULP

Filed Aug. 6, 1937

2 Sheets-Sheet 2



Fig. 4



Fig. 5

BY

LOREN V. FORMAN  
*[Signature]*  
ATTORNEYS

INVENTOR.

## UNITED STATES PATENT OFFICE

2,207,218

PROCESS FOR REMOVAL OF DIRT FROM  
PULP

Loren V. Forman, Munising, Mich., assignor of  
one-half to The Munising Paper Company,  
Munising, Mich., a corporation of Ohio

Application August 6, 1937, Serial No. 157,767

1 Claim. (Cl. 92—28)

This invention relates to a process for the removal of dirt from pulp for making paper.

It is the object of this invention to provide a novel process for the separation of dirt from paper pulp by hydraulic classification. In the definition of "dirt" there is included rust, scale, sand, mineral dirt, particles of digester lining, lime particles, knots, uncooked chips, bark specks, shives and fiber bundles. All suspended material except the individual pulp fibers is classified as "dirt."

It is an object of this invention to utilize low consistencies of paper pulp in which sufficient differentials in settling rates are secured between dirt and pulp to provide a basis for separation.

It is an object of the invention to utilize a uniform velocity of a rising water column at such speed as to prevent fibers from passing downwardly into a receiver, yet permitting dirt to fall into the receiver so that by a carefully controlled rising current in the sorting column and by using very low consistencies, an efficient removal of fine dirt is obtained.

It is a further object to provide for using this process with classifiers and rifflers using the riffler as the primary settling chamber and equipping the riffler lines with hopper bottoms and sorting columns for continual separation and removal of knots and dirt to settling chambers either with or without continuous means for discharge therefrom.

It is an object of this process to dilute the pulp to the proper consistency followed by a combination of riffling sedimentation and hydraulic classification to secure separation of all foreign bodies from the cellulosic fibers.

It is an object to provide this process so that it is applicable to all types of pulp and at any points in the system from the digesters to the paper machines.

It is a further object to provide for the addition to the foregoing a process of the use of secondary water and means of giving stepwise classification prior to the final classification in the sorting column in which the foregoing process is utilized.

It is the object of this invention to apply the discovery that for each type of dirt there is a maximum consistency above which no settling is possible and no removal can be accomplished.

It is an object of this invention to employ consistencies that are relatively low so that foreign materials heretofore not commonly classified as dirt and not considered removable by hydraulic classification can be removed. It has been found, when practicing the teachings of this invention, that pulp can be supplied to the classifier at consistencies in the range of 0.1 per cent to 0.25 per cent and from 0.02 per cent up. Consistency is defined as pounds of fiber in one hundred pounds

of the suspension consisting of water, fibers and/or other material suspended in it.

It is an object of this invention to provide for actual separation of dirt from fibers in the classifier at consistencies from zero to that at which the pulp is introduced into the classifier.

It is a further object to reduce the cost of wood as hereinafter explained.

Referring to the drawings:

Figure 1 is a diagrammatic view in side elevation of the apparatus for the practice of this invention as applied to a riffler channel.

Figure 2 is a section on the line 2—2 of Figure 1, looking in the direction of the arrows.

Figure 3 is a view similar to Figure 1 showing a modified form for the introduction of secondary water and for the practice of stepwise classification in the hopper prior to final classification in the sorting column.

Figure 4 is a top plan view thereof.

Referring to the drawings in detail, 1 designates the inlet of stock pulp and dirt passing through the horizontally disposed channel 2 of a riffler. 3 indicates the level of the stock. The bottom of this riffler channel 2 is provided with one or more hoppers 4. The region of entry of the dirty stock is in the zone designated generally at 5. At this point the dirty stock enters in the pyramidal or conical hopper 4. As the dirty stock passes from the channel 2 into this region 5, its forward velocity decreases due to an enlarging cross section of the body of stock as it passes over and into the hopper 4. At the same time the heavier particles settle toward the bottom of the hopper 4 and then enter the sorting column 6 which is of restricted cylindrical area and communicates with the bottom of the hopper 4.

In this sorting column 6 is introduced a rising current of water through the pipe 7 which is equipped with a suitable control valve. This water is introduced preferably tangentially to secure enough spiral motion to produce a uniform rising current across the cross section of the sorting column 6. Its motion is relatively very slow and does not produce any separation by centrifugal force. The amount of water added is carefully regulated so that no good fibers will settle, yet any material having a higher settling

velocity than the good fibers will settle through to the water filled receiver 8 below. Such material is introduced through the hopper 9 and past the valve control 10. The dirt so deposited in the receiver 8 may be intermittently or continuously conveyed away. There are no currents below 10 except as water is displaced by dirt in the receiver 8.

The settling rates of the dirt materials are determined as a function of the consistency of the

- pulp suspension. It has been found that by going to low consistencies sufficient differentials in settling rates between the dirt and pulp are obtained to serve as a basis for separation. The 5 amount of water introduced into the sorting column or settling tube 6 is just sufficient to prevent fibers from passing down into the receiver, yet not too great a flow to permit dirt to fall through it into the receiver 8.
- 10 This process results in the dirt-free pulp making its exit as clean stock through the region generally designated 11 at the top of the outgoing side of the hopper 4 into the continuation of the riffler 2. This process has been found to 15 work very satisfactorily as a knotter, possessing several advantages over the rotating cylindrical knot screens used in this art.

It is also optional to use baffles in the riffler channel 1 above the classifier hopper 4 to deflect 20 the pulp stream downwardly into the classifier. These baffles 1a may extend downwardly into the upper portion of the hopper, or where the classifiers are used independently, they may be located in the upper portion of the hopper. One of the 25 preferable locations is indicated in Figures 1 and 2.

The method of introducing and removing pulp from the classifier, of course, can be employed in the case of a conical hopper operated independently of a riffler. In that event, the pulp is introduced centrally either at the surface, or at 30 some submerged point along the axis of the cone, in such a way that the direction of flow at the point of introduction is radial at that section. In 35 such a case the clean stock overflows the top circumference of the cone and is collected and carried away in a circular trough or launder.

Referring to Figures 1 and 2, the valve 10 is wide open during normal operation. If a single 40 receiver 8 is used, the valve 10 is closed tightly momentarily while the receiver is emptied and immediately opened wide when normal operation is resumed. When two receivers are provided and operated so that one is emptied while the 45 other fills, an additional swing gate is provided to divert the dirt to the proper receiver and seal off the other for emptying. In this case, as when continuous removal of dirt from the receiver is used, the valve 10 is merely an emergency valve 50 to permit repairs to the receiver without loss of pulp. For intermittent operation of a single receiver, the piping connections have been drawn schematically as indicated on Figure 2 by the legends. To empty the receiver, valve 10 is 55 closed, the discharge valve is opened, the water valve is opened to wash out the dirt, and the air vent is opened. When the dirt has all washed out, the discharge valve is closed and the water valve and air vent closed after the receiver is full. 60 of water, whereupon valve 10 is reopened.

This classifier has the advantage of being able to separate small particles of heavy dirt which ordinarily pass through a knot screen easily and may pass through the flat screens if the particle 65 size has been sufficiently reduced by the time it reaches that point in the system. There is no fiber loss in the classifier as each knot or dirt particle is washed free of stock as it falls into the settling column 6 against the rising current of water.

Another advantage of this classifier process for removing knots is that there is no tumbling about of the knots as in the screen type knotter which tends to break up bark dirt and some 70 knots, thereby producing small fragments which

are very difficult to remove in subsequent operations.

By carefully controlling the rising current from the pipe 7 in the column 6, a very efficient removal 5 of fine dirt is obtained so that when the classifier is used in series with a riffler there is produced a cleaner pulp than the conventional riffler and fine screen in series. A microscopic study has revealed that much of the fine dirt can pass through fine screen slots more easily than can the 10 fibers themselves. The minute specks of high density dirt, which usually have quite regular shapes, are not removable by screening when their smallest dimension is less than the width of the screen slot, yet they are readily removed by 15 the classifier.

The fine "wood dirt" particles having settling velocities very close to those of fibers are most difficult to remove by classification, yet this process removes this material efficiently even in the 20 size range encountered in stock that has already passed a ten cut screen plate. This method of removal of this process does not possess the disadvantage encountered in vibrating flat screens to break up brittle, friable dirt to the point 25 where it passes through the slot into the system.

This classifier process has a distinct advantage over flat screens in the cost of operation and maintenance. It has been found that when the classifiers and rifflers are combined, utilizing the 30 riffler area as the primary settling chamber and equipping the riffling lines with the hopper bottoms and sorting columns of this invention for continuous separation and removal of knots and dirt, it is possible to get the result described 35 herein.

This process does not employ the centrifugal principle in any way. The only reason for a rotating of the sorting column to any degree is to secure a uniform distribution of the water so 40 that there will be a uniform vertical current at all points in the cross section of the sorting column 6.

This process permits of the further advantage 45 that it permits of continuous operation as distinguished from intermittent operations of present riffling processes. The present process provides for positive separation of dirt from fibers which eliminates stock losses. It permits of the removal of finer material than is generally included in the ordinary definition of "dirt."

Turning to the form shown in Figures 3 and 4, the hopper 4 is provided with a plurality of spaced collars 12 crimped to conform with the inside of the hopper and having projecting edges 55 12a, as shown in Figure 4, of sheet metal, steel plate, or other suitable material which are fastened in place in planes approximately parallel to the top of the conical or pyramidal hopper 4. The collars are made in sections of a cone or 60 pyramid depending upon the shape of the classifier hopper 4, so that the separated material will slide down over the upper surface of each collar 12 rather than deposit upon it.

The secondary water is distributed through shower pipes built in either square or circular shape to fit under the respective collars 12. These pipes are indicated 13 and are fed by supply pipes 14 equipped with suitable control valve. 70 The secondary water so delivered is relatively small in volume and will serve to reduce the consistency of the body of pulp and dirt and provide an upward sorting current in the regions of restricted cross section formed by the collars 75

12, particularly where the pulp slides down the collars 12 and off the edges 12a.

With the proper adjustment of the secondary water, stepwise classification is obtained which 5 is more efficient in many cases than classification by the one sorting column 6 alone. Especially where a cone shaped hopper is used, the cross section is restricted by a flat wheel or a ring with spokes instead of the ring alone.

10 Another variation of the apparatus for practicing this process is the use of perforated plates having the area of perforations suitably less than the total cross sectional area.

#### Consistencies

15 The primary basis upon which this process has been developed was the discovery that for each type of dirt there is a maximum consistency above which no settling is possible and no removal can be accomplished. At the present time 20 it is understood that consistencies of 0.3 per cent to 0.5 per cent are used in connection with the separation of dirt, but these consistencies will not permit of the separation of material not commonly classified as dirt but which are very injurious if they remain in the paper pulp. It is 25 possible by the employment of this process to utilize consistencies below this range, which results in removing smaller foreign materials heretofore not commonly classed as dirt and not considered removable.

30 Preferably this invention has been practiced by supplying pulp to the classifier at consistencies of from 0.1 per cent to 0.25 per cent, but consistencies from 0.02 per cent up are feasible. Furthermore, within the classifier the consistency 35 becomes progressively lower toward the bottom of the hopper 4. This is due to the addition of secondary water through the pipes 13 and the water from the pipe 7 delivered to the sorting column. At the bottom of the sorting column 6, a complete separation of fibers and dirt has 40 been accomplished and hence the consistency at that point is zero. Consistency is defined as pounds of fiber in one hundred pounds of the 45 suspension consisting of water, fibers and/or other materials suspended in it.

Actual separation of dirt from fibers in the classifier takes place at consistencies from zero 50 on up to that at which the pulp is introduced into the classifier.

#### Effect on the preparation of the wood for cooking

55 The result of this invention in being able to remove all types of dirt, including bark specks, from the cooked pulp makes possible the complete elimination, or at least a material reduction, in the amount of mechanical cleaning done in the wood room where wood is prepared and chipped before cooking. This means a material reduction in equipment such as knife barkers, knot borers, splitters, barking drums, etc. This 60 in turn reduces labor costs, permits the manufacture of more uniform chips and reduces or eliminates losses of wood due to waste in the cleaning process. The latter often amounts to five or ten per cent of the wood purchased. Wood costs are the largest single item of cost in the production 65 of paper containing wood pulp.

This invention also eliminates the necessity for

70 mills making fine paper paying premium prices for clean wood.

It is further possible through the use of this process to cook unbarked wood which eliminates the barking process in mills which do their own 5 barking and eliminates the expense of buying peeled wood where that is practiced.

It is further possible by this process to reduce wood and bark to pulp form, reduce the pulp and associated materials suspended in the water to 10 the consistencies indicated and to make the elimination by this hydraulic classification process of all of the foreign material without going to the expense of pre-preparing the raw material by the expensive methods heretofore practiced, particularly in the making of fine papers.

There are two other important applications of this process. The first is merely a refinement in the use of the classifier in conjunction with a riffler in which instead of equipping the entire 20 length of a riffler channel with a series of hopper bottoms and classifiers, only one unit is installed, probably but not necessarily at the discharge end of the channel, and the dirt settled in other portions of the channel delivered to it for final separation from adhering pulp. This settled material may be delivered to the classifier by any type of mechanical conveyor, such as a slow moving drag scraper conveyor or screw conveyor, or by 25 pneumatic or hydraulic means.

The other application is the use of this classifier to separate clean pulp from dirt in the rejects from any pulp screening operation. Such rejects, 30 usually known as tailings or screenings, commonly are rich in dirt, containing as a rule less pulp 35 than dirt. However, if the clean pulp is not reclaimed from the rejects, the economic loss is considerable. Likewise, in cases where the conventional type of rifflers are used and cleaned intermittently, this classifier can be employed to operate on the settled material as it is washed 40 out to free it of clean pulp.

It will be understood that the term "riffler" in its broadest sense includes not only the conventional type consisting of channels containing numerous baffles over which the pulp must flow, but all types of settling channels and basins, whether containing several baffles, few baffles, or no baffles at all.

It will be understood that I desire to comprehend within my invention such modifications as come within the scope of the claim and the invention.

Having thus fully described my invention what I claim as new and desire to secure by Letters 55 Patent is:

The process of separating dirt from wood pulp in a water suspension, which comprises diluting the stock to a consistency of .02% to .25%, flowing said suspension in a horizontal plane across a settling chamber, allowing the dirt and heavy stock to settle, introducing a rising current of water at different depths in the settling chamber, thereby progressively sorting said dirt from the fibers by moving the fibers upwardly while the dirt settles, and introducing water tangentially to the settling chamber above the point at which said water enters the settling chamber, whereby the settling material is treated to a uniformly rising current of water to remove any remaining fibers from the dirt.

70 LOREN V. FORMAN.